

J. P. COPLAND,  
FURNACE AND LINING THEREFOR.  
APPLICATION FILED AUG. 10, 1918.

1,341,299.

Patented May 25, 1920.



FIG. 1.



FIG. 2.

FIG. 3.

INVENTOR,  
James P. Copland  
By Hull, Smith, Brock & West,  
Attys.

# UNITED STATES PATENT OFFICE.

JAMES P. COPLAND, OF SOUTH EUCLID, OHIO, ASSIGNOR TO THE ELYRIA IRON AND STEEL COMPANY, OF CLEVELAND, OHIO, A CORPORATION OF OHIO.

## FURNACE AND LINING THEREFOR.

1,341,299.

Specification of Letters Patent. Patented May 25, 1920.

Application filed August 10, 1918. Serial No. 249,230.

To all whom it may concern:

Be it known that I, JAMES P. COPELAND, a citizen of the United States, residing at South Euclid, in the county of Cuyahoga and State of Ohio, have invented a certain new and useful Improvement in Furnaces and Linings Therefor, of which the following is a full, clear, and exact description, reference being had to the accompanying drawings.

This invention relates to furnaces and especially to such furnaces as are subjected to high degrees of temperature for long periods as in metallurgical works, although not limited to this use as I shall hereafter show. The object of the invention is the provision of a furnace of such construction and lined with such material as to withstand elevated temperatures practically indefinitely without burning out, warping, cracking or otherwise deteriorating as has always heretofore been the case.

The essence of my said invention consists in lining such a furnace with a metallic alloy containing a preponderance of one or more iron group metals together with a considerable percentage of chromium, with or without other metals of the chromium group. By iron group metals I means the metals iron, manganese, cobalt and nickel; and by chromium group metals I means the metals chromium, molybdenum and tungsten.

The iron group metal which I preferably employ in preponderating amount is iron owing to its comparative cheapness, though nickel appears to be equally effective in most cases and its use in considerable proportion is impeded only by its high cost. I frequently, and in fact preferably, alloy the iron with a small proportion of nickel since this mixture affords a considerable elevation of the melting point, decreases the tendency to warp on heating, and affords a degree of resistance to oxidation. I ordinarily employ nickel up to a proportion of about 4 or 5 per cent. although its use up to about 20 per cent. produces a superior alloy.

Manganese may also advantageously be added since it possesses a peculiarly marked effect in elevating the melting point and increasing the hardness of iron and its alloys. It also has a beneficial influence in preventing oxidation of the iron. I have generally employed the same only in small quantities, for example about 1.5%, but do not confine myself thereto.

The main advantage imparted by the chromium flows from the adherent and impervious character of its oxide which serves as a protective coating shielding the metal therebeneath; although it is also of advantage in raising the melting point of the alloy, decreasing its coefficient of expansion, and reducing its tendency to warp and twist with changes of temperature. I preferably employ this material within the limits of 10 and 40 per cent. by weight, since below 10 per cent. its shielding effect becomes decreased and the melting point of the alloy becomes too low, while above 40 per cent. the cost of the alloy is rendered unnecessarily high.

Tungsten may also be used in the alloy and has a decided value in increasing the melting point, although its liability to oxidation indicates that its proportion should be kept small; I preferably employ about one per cent.

As an example of a very satisfactory material for use in my invention I will cite the following analysis:

|            |       |    |
|------------|-------|----|
| Silicon    | 17    |    |
| Sulfur     | .026  |    |
| Phosphorus | .042  | 85 |
| Carbon     | .66   |    |
| Vanadium   | .18   |    |
| Tungsten   | .92   |    |
| Manganese  | 1.47  |    |
| Nickel     | 4.87  | 90 |
| Chromium   | 18.60 |    |
| Iron       | 72.95 |    |

Such an alloy will not warp or twist even with repeated heating; will not melt or even soften at any temperature up to the melting point of iron; will not become oxidized at any temperature short of its own melting point; and has a coefficient of expansion within the limits of those of firebrick wherefore it does not tend by its changes in size to wreck the casing or shell with which it is ordinarily surrounded.

Such an alloy is most conveniently made in the electric furnace, but the particular method of making the same has no bearing upon the present invention, since it will be understood that the alloy could perfectly well be made by melting the pure constituents by suitable means such as in an electric vacuum furnace. Furthermore, the alloy is preferably formed in the desired shape for

use by casting in a suitable mold, since rolling is impossible, at least when cold, and machining is very slow and expensive. The material may either be cast in the completed 5 form of a finished furnace lining or may be made in the form of plates which are subsequently bolted or otherwise secured together; and may either expose its outer side to the air or to other gases, or may be surrounded 10 and backed up by firebrick, magnesia, asbestos, gypsum, sand, or other suitable or convenient material.

This construction may be used for muffle 15 furnaces, crucible furnaces, annealing furnaces, re-heating furnaces, heat-treating furnaces, hardening furnaces, rivet heaters, welding and forging plants, steam boiler furnaces, bakers' furnaces, and all other types of heated devices either for metallurgical 20 plants, iron works, glass works, pottery works, blacksmith shops, garages, shipyards, repair shops, bakeries, or other places where heating is done, and may be used with gas, coal, coke, oil or electricity.

25 In the drawing accompanying and forming a part of this application Figure 1 is a cross-sectional view through a simple small furnace embodying my invention; Fig. 2 is a longitudinal sectional view of a part of a 30 different type of furnace constructed in accordance with my invention; and Fig. 3 is a cross-sectional view of another type of furnace constructed in accordance with my improvements.

35 Referring first to Fig. 1, 1 represents the metallic lining which is here shown as cast in a single piece and having at one side the aperture 2; 3 represents a casing or shell of brick or the like structural material built 40 therearound and preferably spaced from the exterior of the lining to provide a space 4 which is filled with some soft refractory packing 5 such as magnesia, sand, gypsum, asbestos or the like, which serves to fill any 45 inequalities in the adjacent walls, to conserve the heat inside the furnace, to shield the casing from undue temperature, and to form an elastic or yielding layer which shall take up strains and permit the relative 50 expansion and contraction of the parts without injury thereto. The casing 3 is shown as provided with an aperture 6 in alinement with the aperture 2 and receiving a tube 7, which may conveniently be of the same material 55 as the lining 1 and permit the admission of the heating element, which may be incandescent gases produced by a combustion exterior of the furnace or may be any inflammable mixture to be burned inside the 60 furnace.

In case the furnace be of small size it is possible and in fact customary to close the opening more or less by means of firebrick so piled as to permit the escape of any waste 65 gases or combustion products, but in case the

furnace be of larger size it is sometimes convenient to provide a more elaborate closure, as will be well understood by those skilled in the art. In an electrically heated furnace no opening is necessary for the discharge of any burned gases, but only a suitable aperture or apertures for the passage of the conductors.

In Fig. 2 I have illustrated a muffle furnace wherein 15 represents a furnace lining as hereinbefore described, which is here shown integral with the inlet tube 16 and with the flue lining 17. The furnace lining is here shown as of double-wall construction providing a muffle chamber 18 whose top 75 80 may be either open so that the hot gases can sweep therethrough or closed by a lid 19, either integral or removable as desired. This muffle furnace is as before provided with a shell 3 and with a refractory pack- 85 ing 5.

In Fig. 3 I have shown a furnace of larger size suitable for a great number of purposes such as annealing glass or metal articles, heat treatment, cementation, case hardening, etc. In this embodiment the lining is composed of a plurality of separate plates 20—20 of the resistant metal herein described, each of the plates being formed with marginal flanges 21—21 and the flanges 90 95 of adjacent plates being suitably fastened together as by bolts or pins. It will also be understood that the flanges of adjacent plates can be so fashioned as to interfit, thus dispensing in whole or part with the necessity of independent fastenings. The various plates can be made of any suitable or convenient shape, but are preferably substantially standard in shape and size so that a large number of different furnaces can be 100 105 built with a small number of patterns. This lining as before, is preferably surrounded by a shell 3 and packing 5, and can be heated in any suitable manner as heretofore explained.

110 It will be understood that these drawings are illustrative only and not limiting; that the forms and constructions in which my invention can be embodied are almost limitless; that I do not restrict myself to a construction involving a spaced outer shell in combination with the lining and an intervening space to be filled with unformed material, but merely present that as being a cheap and satisfactory construction; and 115 120 that in general I do not limit myself except as recited in the claims hereto annexed or rendered necessary by the prior state of the art.

Having thus described my invention, what 125 I claim is:—

1. A cast metal furnace lining consisting of an alloy containing from 70 to 75 per cent. of iron and 15 to 25 per cent. of chromium, the remaining consisting prin- 130

cipally of other metals from the iron and chromium groups.

2. In a device of the character described, the combination with a firebrick casing, of

5 a cast metal lining consisting principally of a metal or mixture of metals of the iron group alloyed with chromium, the iron group metal being preponderant and the alloy having a coefficient of expansion with-

10 in the limits of that of firebrick.

3. A cast metal furnace lining consisting approximately of manganese 1½ per cent., nickel 5 per cent., tungsten 1 per cent., chromium 20 per cent. and the remainder prin-

15 cipally iron.

4. A furnace having incorporated therein

a multiple walled lining composed of a metallic alloy containing one or more iron group metals alloyed with 5 to 40 per cent. of chromium.

20

5. A cast metal furnace lining composed of an alloy comprising the major portion of iron, and the remainder of metals from the iron and chromium groups.

6. A cast metal furnace lining consisting 25 of an alloy containing 70 to 75 per cent. of iron, 15 to 25% of chromium, and the remainder of a metal from the iron group.

In testimony whereof, I hereunto affix my signature.

JAMES P. COPLAND.